

1

3,493,504

## FIBER LUBRICANT

Herman T. Buckley, Cincinnati, Ohio, assignor to Emery Industries, Inc., Cincinnati, Ohio, a corporation of Ohio  
 No Drawing. Filed June 27, 1966, Ser. No. 560,862  
 Int. Cl. D06m 15/44, 13/34  
 U.S. Cl. 252—8.8

10 Claims

## ABSTRACT OF THE DISCLOSURE

This invention relates to a fiber lubricant and more particularly to fiber lubricant compositions comprising as a lubricant base the condensation product of alkanolamines and fatty acids, as an emulsifying agent, a polyoxyalkylated fatty alcohol, and as a rust inhibitor, an aliphatic di-carboxylic acid salt.

## BACKGROUND OF THE INVENTION

This invention pertains to the textile art and more particularly to the fiber lubricant art. In the textile field, it is necessary to prepare the fibers prior to their processing so that they have the proper balance of what is called fiber to metal and fiber to fiber lubricity. The fiber to metal lubricity is needed in order to prevent excessive breakage of the fiber during its processing into yarn in the carding and spinning operations. The fiber to fiber lubricity must be properly controlled in order to impart to the fibers cohesiveness properties which will prevent them from slipping and sliding during the carding and spinning operations. Also, in the fiber art, particularly in the carpet field, it is essential that the fiber lubricant also impart to the fibers which are processed into carpet, low soiling characteristics. In the past, the materials which have been found most satisfactory as fiber lubricants have been cationic materials such as fatty imidazoline salts. Although the cationic materials impart good anti-friction and low soiling properties to the fiber, they are very corrosive in nature and their use frequently results in the deposition of corrosion bodies on the yarns. The corrosion or rust comes from the non-stainless steel machinery which has been exposed to the conventional cationic lubricant. Some improvement in the cationic lubricants has been obtained by the addition of rust inhibitors to the cationic emulsions used; however, even with rust inhibitors, the cationic lubricants have not been able to provide entirely satisfactory results.

The fiber lubricants of the present invention have overcome the above-noted problems of the past connected with cationic fiber lubricants by providing in a basic formulation, a material which in addition to being non-corrosive imparts to the fibers excellent lubricity and low soiling characteristics.

## DESCRIPTION OF THE INVENTION

The fiber lubricant compositions of the present invention comprise (1) the condensation product of an alkanolamine and a fatty acid, (2) a polyoxyalkylated fatty alcohol, and (3) an aliphatic dicarboxylic acid salt.

The condensation product is prepared from an alkanolamine having the general structure



wherein  $R_1$  and  $R_2$  are selected from the group consisting of hydrogen and lower hydroxy alkyl radicals and wherein at least one of  $R_1$  and  $R_2$  is a lower hydroxy alkyl radical, and a  $C_9-C_{24}$  fatty acid. The fatty acid may be either saturated or unsaturated, although saturated acids are preferred. Examples of alkanolamines which may be used

2

are ethanolamine, diethanolamine, propanolamine, di-propanolamine, isopropanolamine, di-isopropanolamine, hydroxy butyl amine, and the like. Among the fatty acids which may be used are stearic, palmitic, myristic, and oleic acids. The composition of the condensation product is dependent upon the amount of amine and acid used in its preparation but generally consists of a combination of mono-esters, di-esters, amides and ester-amides, predominantly the latter. The ratio of amine to fatty acid varies depending upon the functionality of the amine, but preferably about two equivalents of acid are used for every one equivalent of amine.

The polyoxyalkylated fatty alcohols which are employed as emulsifying agents in the compositions of the present invention should conform to the structure



wherein  $R_2$  is a lower divalent alkyl radical having from 2 to 3 carbon atoms,  $R_1$  is a higher hydrocarbon radical having from 6 to 18 carbon atoms, and  $n$  is an integer from 1 to 40, preferably from 20 to 25. The polyoxyalkylated fatty alcohols may be made by reacting such alkylene oxides as ethylene oxide or propylene oxide with lauryl alcohol, cetyl alcohol, myristyl alcohol or the like. The term "lauryl" as used herein is intended to include the fatty hydrocarbon chains of fatty alcohols derived from coconut fatty acids. Thus lauryl alcohol would include a mixture of alcohols having chain lengths of from 6 to 18 carbon atoms but predominantly 10 to 14 carbon atoms in length.

The third essential ingredient of the present fiber lubricant compositions is an aliphatic dibasic acid salt which is used as a rust inhibitor. The aliphatic dibasic acid salts may be prepared from aliphatic dibasic acids having from about 6 to 12 carbon atoms including adipic, azelaic, sebacic, and dodecanoic acids. The metal component of the salt should be an alkali metal, preferably potassium or sodium and may be either mono or di-substituted although the former is preferred. Examples of suitable dibasic salts which may be used are di-potassium azelate, mono-potassium azelate, disodium azelate, mono-sodium azelate, di-potassium adipate, di-potassium sebacate, and mono-potassium sebacate.

In the formulation of the fiber lubricants of the present invention, the condensation product of an alkanolamine and a higher fatty acid should constitute from 50 to 90% of the lubricant. The polyoxyalkylated fatty alcohol emulsifying agent should constitute from 9 to 40% and the aliphatic dibasic acid salt should constitute from 1 to 10% of the lubricant composition.

The fiber lubricants of this invention may be prepared by melting the alkanolamine-higher fatty acid condensation product and the polyoxyalkylated fatty alcohol, which are usually solids, and blending the two materials together. Thereafter, the aliphatic carboxylic dibasic acid such as azelaic acid, is intermixed with the blend and after it has melted into the blend, an alkali solution of either potassium hydroxide or sodium hydroxide is added to saponify the acid and produce the aliphatic carboxylic dibasic acid salt. The fiber lubricants are ordinarily used in the form of an aqueous emulsion and thus water is usually added to the melted blend in an amount which gives the dilution desired, and stirring is continued until a completely emulsified and homogenized blend is obtained, after which the resulting emulsion is cooled.

In one preferred embodiment of the present invention the fiber lubricant is prepared by blending together 20 weight percent of the condensation product of di-ethanolamine and stearic acid which is prepared by reacting the stearic acid with the amine at a ratio of about two moles of acid to one of amine, the product being principally 2-(N-hydroxy ethyl) stearamido ethyl. 4.5 weight percent

of ethoxylated lauryl alcohol, 0.5 weight percent mono-potassium azelate and 75% by weight water. In this particular embodiment of the present invention, the relative amounts of the three active ingredients of the composition which can be used is rather restricted. The di-ethanolamine-stearic acid reaction product must constitute from 70 to 90% by weight of the three component lubricant mixture, the ethoxylated lauryl alcohol must constitute from 10 to 30%, and the mono-potassium azelate must constitute from 1.0 to 5% by weight of the basic lubricant composition.

The fiber lubricant of the present invention may be applied to the fibers either before or after they have been dyed by spraying the lubricant composition, usually in water-diluted form, onto the fiber prior to the processing of the fiber, or the lubricant may be incorporated in the aqueous rinse which is used upon the fiber after the fiber has been dyed. The fiber absorbs the lubricant from the rinse water in the latter instance.

The following examples are provided to further illustrate the invention but are not to be construed as limitative of the scope thereof:

#### EXAMPLE I

A lubricant base was prepared in the following manner: A reaction vessel was charged with 105 parts of di-ethanolamine and 540 parts of stearic acid of the conventional triple press grade. These two reactants were heated at 225° C. until two mole equivalents of water had been removed and the acid value was reduced to 3.8. The reaction product was then cooled under vacuum.

#### EXAMPLE II

A fiber lubricant was prepared by melting and then blending together 200 grams of the reaction product of Example I and 45 grams of a polyoxyalkylated fatty alcohol, polyoxyethylene (23) lauryl ether. To the blend was added 3 grams of azelaic acid which was melted into the blend and then 2 ml. of a 50% solution of potassium hydroxide (50 weight percent KOH) was added to the blend as it was being stirred. While the melted blend was still hot, 750 ml. of water were added and the blend was stirred until a completely emulsified and homogenized product was obtained, and then the resulting material was cooled.

#### EXAMPLE III

The corrosion resistance of the fiber lubricant prepared in Example II was determined in the following manner: A metal non-stainless steel pad thoroughly cleaned with acetone was placed in a jar after which it was covered with the lubricant of Example II. The jar was then closed and stored for one week at room temperature. Three additional tests were conducted in this same manner except that in one a 10% solution of the material of Example II prepared by diluting the lubricant of Example II at a 90:10 ratio of water to lubricant was used, in the second a conventional ionic type fiber lubricant containing as the active cationic agent, distearyl imidazoline, in an aqueous solution in which the active material was approximately the same strength as the 90:10 diluted fiber lubricant described above was used, and the third was a blank test in which water alone was used.

Fiber lubricant used: Corrosive activity after one week

|                               |       |                                                                      |       |                                                                  |       |                                                                  |       |                                                |
|-------------------------------|-------|----------------------------------------------------------------------|-------|------------------------------------------------------------------|-------|------------------------------------------------------------------|-------|------------------------------------------------|
| Fiber lubricant of Example II | ----- | No emulsion discoloration or 10% solution of lubricant of Example II | ----- | No emulsion discoloration or 10% solution of cat-ionic lubricant | ----- | No emulsion discoloration or 10% solution of cat-ionic lubricant | ----- | Severe emulsion discoloration and pad rusting. |
| Water                         | ----- | Severe pad rusting and water discoloration.                          |       |                                                                  |       |                                                                  |       |                                                |

#### EXAMPLE IV

The lubricity of a fiber treated with the fiber lubricant of the present invention was determined by impregnating a fiber sample with an emulsion of the fiber lubricant of Example II which was diluted at a 95:5 water to lubricant ratio giving an aqueous emulsion having 1 1/4% active lubricant ingredients. The impregnation was performed by passing the yarn sample through a bath of the dilute emulsion and then squeezing the yarn with a hand wringer and drying on a non-absorbent surface. About 100% wet pick-up of the solution was accomplished following this procedure. The fiber to metal lubricity was measured by attaching the lubricated yarn to a gram scale, then passing it under but in contact with a steel wheel and finally threading it over a free pulley to which is attached at the other end of the yarn a weight, i.e., 50-gram weight. The steel wheel was rotated against the fiber to determine the frictional force, which was read from the gram scale. The yarn treated as described above and tested for friction with this apparatus showed a fiber to metal friction of 68 grams. An untreated yarn was tested for friction and showed a fiber to metal friction of 72 grams.

#### EXAMPLE V

The soil resistance of the fiber lubricant of Example II was determined in the following manner: Yarn samples of polypropylene, acrylic, nylon, wool, and polyester each weighing 2.5 grams were thoroughly scoured with a commercial nonionic detergent, ethoxylated nonyl phenol and soda ash, then rinsed in distilled water and rinsed in both ethyl ether and isopropanol. The emulsion of Example II was dissolved in a 90:10 ethyl ester-isopropanol solution and then applied to the various yarn samples in an amount of 0.5% active lubricant ingredients (based on the weight of the yarn) and was worked into the yarn. The yarn samples were cut into 1 1/2- to 2-inch strips and were tightly placed parallel to each other on a glass plate covered with gray cardboard. A second plate covered with black cardboard except for an opening through which readings could be taken was placed over the yarn samples. The plates were securely clamped together with rubber bands and the resulting "sandwich" was then placed over an opening on a Gardner Reflectometer and readings were taken on the green filter only (66.2 standard). A standard or blank sample of each of the yarns was also prepared in which the straight ethyl ether-isopropanol solution was applied to the yarns. After their reflectance was measured, the individual strips were then placed in pint jars containing (1) ten stainless steel balls 1/4 inch in diameter and (2) two grams of artificial soil consisting of 0.1% carbon black, 1.7% rottenstone, and 98.2% sodium sulfate as a carrier. The jars containing the yarn and artificial soil were then securely clamped in a Launder-Ometer and tumbled for fifteen minutes at 42 r.p.m. per minute. The yarn strips were then transferred to dusting cans which were 4 1/2 inches in diameter and 4 3/4 inches high and have 1/8-inch holes 1/2 inch apart at the top and bottom, 1 inch apart horizontally and 1/2 inch apart vertically on the sides. Ten clean steel balls 1/2 inch in diameter were added to the cans and the cans were tumbled in the Launder-Ometer for thirty minutes after which their reflectance was again measured with a Gardner Reflectometer. The yarn soiling is determined in terms of a soiling index or percent increase or decrease in the soiling of the treated as compared with the untreated yarn. The soiling index is obtained by use of the following formula:

$$\text{Soiling Index} = \frac{\Delta^{RT}}{\Delta^{RU}} \times 100$$

$\Delta^{RT}$  = change in reflectance of treated yarn.

75  $\Delta^{RU}$  = change in reflectance of untreated yarn.

The results obtained with the various fibers are shown in the table below:

| Fiber:        | Percent increase or decrease in soiling |
|---------------|-----------------------------------------|
| Polypropylene | -10.2                                   |
| Acrylic       | +28.7                                   |
| Nylon         | -1.4                                    |
| Wool          | -1.0                                    |
| Polyester     | +4.0                                    |

As may be seen from the above results, the soil resistance properties of propylene, nylon, and wool are enhanced by the use of the fiber lubricant of the present invention. The results obtained with acrylic and polyester fibers may superficially appear to be objectionable, however, fiber lubricants are essential in the processing of these fibers and the percentage increase in soiling propensities as shown in the above results is actually far less than is normally experienced. Acrylic and polyester fibers generally tend to soil less when used in the untreated form.

What I claim is:

1. A fiber lubricant consisting essentially of  
(a) from 50 to 90% by weight of a condensation product of (i) an alkanolamine having the structure



wherein R<sub>1</sub> and R<sub>2</sub> are selected from the group consisting of hydrogen and lower hydroxy alkyl radicals and wherein at least one of R<sub>1</sub> and R<sub>2</sub> is a lower hydroxy alkyl radical, and (ii) a straight chain higher fatty acid containing from about 9 to 24 carbon atoms;

(b) from about 9 to 40% by weight of a polyoxyalkylated fatty alcohol having the structure



wherein R<sub>4</sub> is a lower alkylene radical having from 2 to 3 carbon atoms and R<sub>3</sub> is a hydrocarbon radical having from 6 to 12 carbon atoms, and n is an integer from 1 to 40; and

(c) from about 1 to 10% by weight of an aliphatic hydrocarbon dicarboxylic acid salt containing from about 6 to 12 carbon atoms.

2. The lubricant of claim 1 wherein R<sub>4</sub> is selected from the group consisting of ethylene and propylene radicals, and n is an integer from 20 to 25.

3. The lubricant of claim 2 wherein said dibasic acid salt is selected from the group consisting of aliphatic hydrocarbon dibasic acid salts of sodium and potassium.

4. The lubricant of claim 3 wherein said condensation product is prepared from the reaction of di-ethanolamine and stearic acid, said polyoxyalkylated fatty alcohol is polyoxyalkylated lauryl alcohol, and said dibasic acid salt is potassium azelate.

5. The lubricant of claim 4 wherein said dibasic acid salt is mono-potassium azelate.

6. The lubricant of claim 5 which comprises from 70-90% by weight of said condensation product, from 10-30% by weight of said ethoxylated lauryl ether, and from 1.0-5.0% by weight of said potassium azelate.

7. An aqueous solution of the lubricant of claim 3.

8. A method for lubricating a textile fiber which comprises applying to said fiber a fiber lubricant consisting essentially of

(a) from 50 to 90% by weight of a condensation product of (i) an alkanolamine having the structure



wherein R<sub>1</sub> and R<sub>2</sub> are selected from the group consisting of hydrogen and lower hydroxy alkyl radicals and wherein at least one of R<sub>1</sub> and R<sub>2</sub> is a lower hydroxy alkyl radical, and (ii) a straight chain higher fatty acid containing from about 9 to 24 carbon atoms;

(b) from about 9 to 40% by weight of a polyoxyalkylated fatty alcohol having the structure



wherein R<sub>4</sub> is a lower alkylene radical having from 2 to 3 carbon atoms and R<sub>3</sub> is a hydrocarbon radical having from 6 to 18 carbon atoms, and n is an integer from 1 to 40;

(c) from about 1 to 10% by weight of an aliphatic hydrocarbon dicarboxylic acid salt containing from about 6 to 12 carbon atoms.

9. The method of claim 8 wherein said condensation product is prepared from the reaction of di-ethanolamine and stearic acid, said polyoxyalkylated fatty alcohol is ethoxylated lauryl alcohol, and said dibasic acid salt is potassium azelate.

10. The method of claim 9 wherein said lubricant comprises from 70-90% by weight of said condensation product, from 10-30% of said ethoxylated lauryl ether, and from 1.0-5.0% by weight of said potassium azelate.

#### References Cited

##### UNITED STATES PATENTS

|           |         |                 |           |
|-----------|---------|-----------------|-----------|
| 2,426,968 | 8/1947  | Farley          | 252-396 X |
| 2,540,678 | 2/1951  | Kelley          | 252-8.8 X |
| 2,628,937 | 2/1953  | Paul            | 252-8.8   |
| 2,730,498 | 1/1956  | Fortress et al. | 252-8.8   |
| 2,857,330 | 10/1958 | Hall            | 252-8.8   |
| 3,029,204 | 4/1962  | Matuszak et al. | 252-396 X |

LEON D. ROSDOL, Primary Examiner

I. GLUCK, Assistant Examiner

U.S. Cl. X.R.

117-139.5; 252-8.9, 8.75, 396